

J. A. HEANY,  
ELECTRIC INSULATION.  
APPLICATION FILED SEPT. 23, 1914.

1,155,812.

Patented Oct. 5, 1915.  
2 SHEETS—SHEET 1.

Fig. 1.



Witnesses.

D. W. Edelin

*[Signature]*

Inventor:

John Allen Heany  
by  
Samuel Goldfarb and M. W. Miller  
*[Signature]*



J. A. HEANY,  
ELECTRIC INSULATION,  
APPLICATION FILED SEPT. 23, 1914.

1,155,812.

Patented Oct. 5, 1915.

2 SHEETS—SHEET 2.



Fig. 2.

Witnesses.

D. W. Edelin

*Frank*

Inventor:

John Allen Heany  
Pawtucket, Rhode Island  
Attest.

# UNITED STATES PATENT OFFICE.

JOHN ALLEN HEANY, OF NEW YORK, N. Y.

## ELECTRIC INSULATION.

1,155,812.

Specification of Letters Patent.

Patented Oct. 5, 1915.

Application filed September 23, 1914. Serial No. 863,123.

*To all whom it may concern:*

Be it known that I, JOHN ALLEN HEANY, a citizen of the United States, residing in the city, county, and State of New York, have invented certain new and useful Improvements in Electric Insulation; and I do hereby declare the following to be a full, clear, and exact description of the invention, such as will enable others skilled in the art to which it appertains to make and use the same.

The invention relates to a new and useful form of insulating sheath or covering for electric conductors and more particularly to a type of insulation produced by the method described and claimed in my prior Patent, No. 1,071,676, dated August 26, 1913, said covering including a foundation thread or filamentary body having applied thereto a body of fibers of asbestos, cotton, jute hemp, or other fibrous material in the form of a matted or felted covering, which fiber-coated filamentary body having applied thereto a conductor to be insulated preferably by winding the said fiber-coated filamentary body about the conductor and working the same down to highly efficient, uniform and homogeneous insulating sheath.

The invention is illustrated in the accompanying drawings, in which:—

Figure 1 is a diagrammatic representation of mechanism for the preliminary covering of a thread or filamentary body with the fibrous insulating material. Fig. 2 is a similar view of apparatus for applying the fiber-coated thread to the conductor. Fig. 3 shows a section of the conductor with the insulating material being applied thereto.

Referring to Fig. 1 of the drawings, 1 indicates a ball, spool or cop of thread or yarn which may be of any desired size, but which is preferably as fine or of as small diameter as the exigencies of the work will permit. Said ball or cop 1 is mounted upon a spindle 2, which may, if desired, be rotated in a direction at right angles to its axis, but which as shown is capable of rotation about its longitudinal axis. As the thread or yarn is paid off of the ball or cop 1, it passes over and around a tension roller 3, thence around a roller 4 which is immersed in a tank 5 containing an adhesive, such as water, glue, paste, albumen, sodium silicate, or any other gelatinous or sticky substance, appropriate to coat the thread or yarn to cause fibrous materials coming in

contact with the thread or yarn to adhere thereto. From the adhesive applying roller 4, the thread passes directly over the doffer of a carding machine or the like, said doffer being represented as a belt 6 of usual and appropriate form, passing over a roller 7 and serving to draw out the elements of the fibrous material in lines parallel with the run of the doffer belt, as will be understood. 60 Beyond the doffer 6, the thread passes around a pulley 17 mounted on the lateral arm of a rotary flier 8 which in turn is rotated on its horizontal axis by a pulley 12 by means of a belt 13, the flier 8 and pulley 70 12 being journaled in a suitable bearing 13'. Carried by the flier 8 is a spindle 9 adapted to receive a spool 18 upon which the fiber-coated thread is wound, rotary motion being imparted to said spool 18 by means of a 75 bevel pinion 10 on spindle 9, which meshes with a bevel gear 11 mounted on the spindle 14 concentric with the axis of flier 8, to the outer end of which spindle 14 is attached a brake drum 15 about which is looped several turns of a cord or rope 16, anchored at its upper ends to a stationary abutment and provided at its lower looped end with a pendant weight 16', the parts being so disposed that as the flier rotates about its horizontal 80 axis, the coaction of pinion 10 with gear 11 will cause the spindle 9 to rotate and wind the thread on the spool 18. The action of the brake drum 15 and its associated cord and weight 16 and 16' admits of the spool 90 18 being rotated with just sufficient force to wind the thread regularly and evenly on the spool 18. By regulating the amount of the weight 16', the degree of tension on the spool rotating mechanism may be nicely adjusted. 95

The apparatus as thus described affords a simple and efficient means for carrying out the first step of the method involved in the present invention, to wit, the preparation of the fibrous material to form the main 100 element of the insulating sheath as a loosely matted or felted mass wound about the relatively light foundation thread for yarn, and preferably secured to the latter by means of a suitable adhesive. It will be understood 105 that the mechanism is merely exemplary and that the operations performed thereby can be produced by other forms of mechanism, or if desired, even by hand.

The operation of the apparatus is as follows: When the thread or yarn is drawn off of the cop 1 and passes around the roller 3 110

and thence through the other parts of the mechanism to the spool 18, the thread is given a rapid rotation about its longitudinal axis, so that when the thread passes in contact with the doffer belt 6, it takes up the straightened threads or fibers of the material carried by the belt and causes said fibers to be wrapped about its body in a loosely matted condition, the fibers however adhering to the thread, first because of the twisting action imparted thereto by the rotation of the thread, and second, because of the cementing effect of the adhesive applied to the surface of the thread by the roller 4. The travel of the thread through the machine may be quite rapid, and by regulating the relative speeds of the doffer 6 and the flier 8, any desired thickness of the fibrous material wound and matted on the thread may be readily accomplished. As the thread leaves the doffer 6, the fibrous coating thereon is more or less fluffy and irregular in appearance, but is nevertheless distributed over the surface of the thread with exceptional regularity, and in passing around the guide roller 17 on the flier head 8, the fibrous coating is more or less compacted, so that when the fiber coated thread is ultimately wound upon the spool 18, it can be laid up in compact regular convolutions. After all of the thread has been unwound from the cop 1, coated with the adhesive and fibrous material and wound upon the spool 18, the latter is removed from the flier head for subsequent use and the operation repeated with another supply of thread and an empty spool 18.

When this or a similar apparatus is employed for coating the foundation thread or filament with asbestos, it is found convenient and preferable to use the cheap, short-fibered asbestos of commerce, which lends itself readily to the carding operation of an ordinary carding machine and is delivered to the doffer in a multiplicity of short filaments which are engaged by the rotating thread and wound and matted thereon in a relatively loose but uniform mass. The thickness of the covering of asbestos fiber on the thread will, as heretofore indicated, depend upon the width of the doffer and the relative speeds of travel of the doffer and the thread. If it is desired to apply a substantially thin but regular coating of asbestos to the thread, a comparatively narrow doffer belt may be employed, or the thread may be fed across the same at a relatively higher rate of speed and correspondingly, if a thicker and heavier coating of asbestos or the like is desired, a wider doffer belt may be employed, or the doffer may be driven at a higher rate of speed, or in the alternative, the thread may be fed more slowly across the doffer. What is true of the asbestos fiber, applies likewise to other fibrous materials which may be employed,

and in any case, the result of the operations is a relatively small foundation thread or yarn of any appropriate material completely covered with a mass of twisted and matted fibers, uniformly distributed over the surface of the thread and affixed to the latter by a suitable adhesive, which fiber-coated thread is wound upon a spool for subsequent use. 70

If it is found undesirable to impart any extra twist to the foundation thread, but nevertheless to cause the thread to take up the fibers from the doffer and dispose the same in a uniform matted layer about its surface, the spindle 2 of the cop 1 may be given a rotary motion in the same direction and at the same speed as the flier head 8, so that the whole body of the thread and its supports will be rotated without twisting any intermediate portion of said thread. 85

To apply the fiber-coated thread to its intended purpose, to wit, as an insulating sheath or covering for conductors, an apparatus such as illustrated in Fig. 2 may be conveniently employed, said apparatus comprising a reel 19 upon which the conductor in the form of a wire, ribbon or the like is wound, a pair of straightening and guiding rollers 21 adjacent the reel, an adhesive applying roller 22 mounted in a receptacle 23 over which roller 22 the wire passes, a rotary flier 24 journaled in a suitable bearing 25 provided with a longitudinal opening through which the wire travels, said flier having one or more studs or pintles 24' upon which are secured one or more spools 18 containing the fiber-coated thread, prepared in accordance with the preliminary method hereinbefore described. The flier 24 is preferably in the form of a pulley driven by a belt 26, as will be understood. Beyond the flier 24, the conductor 20 having the fiber-coated thread wound thereon in spiral convolutions passes over a roller 27 mounted in a receptacle 28 which contains a coating composition and which applies such composition to the fiber-coated thread. 95

If it is desired to water-proof the insulating sheath, the composition contained in the receptacle 28 may consist of paint or varnish, composed of asphaltum, or gums, or resins, or any suitable synthetic plastic resistant substance. If it should be desired to render the insulation fire-proof, then the composition applied by roller 27 may consist of sodium silicate, silicate of lime, kaolin, a metallic oxid, such as oxid of alumina, or a lime product, such as sulfate of lime, or if desired, any admixture of the foregoing ingredients worked up to a gluey cohering consistency and which will ultimately form with the fiber-coated thread a smooth, uniform, coherent, flexible sheath. After leaving the composition applying roller 27, the coated wire is passed through a series of smoothing 115 120 125 130

and finishing devices, which may be of any preferred form and which are effective to smooth and reduce the composite coating to a homogeneous layer of uniform thickness 5 and continuity. As shown in the drawings, said smoothing and finishing devices comprise a series of rotary disks 29 through the center of which the covered wire passes, which disks are driven by belts 30. Upon 10 the rear face of each disk is mounted a pair of bell crank levers 31 having at their free ends clamping jaws 34 which surround the conductor and are held in contact therewith by means of pressure springs 33 disposed 15 between the outer ends of the bell crank levers and the carrying disks. The circular openings formed by the mating grooves in the adjacent faces of the jaws 34 are preferably of successively decreasing diameter in 20 the several devices so that as these jaws are carried around the wire by the movement of the rotary disks, they successively smooth, compact and reduce the coating on the conductor to an enveloping sheath or layer that 25 is uniform throughout and presents a closely adherent shell-like sheath for the conductor. After passing the smoothing and surface-finishing devices, the covered conductor may be subjected to the influence of heat or moisture, as the case may be, for the purpose of 30 setting the coating, as for example, by means of the burner or spraying device 40. The finished wire then passes between guide rollers 41 to a storage reel or bobbin 42. 35 If desired, the foundation thread carrying the fibrous material may be removed from the sheath before the final finishing operation by subjecting the conductor having the fiber-coated thread wound thereon, 40 to sufficient heat to incinerate the thread-like core, without however disturbing the relation of the coating fibers, after which the regular impregnating and finishing operations can be performed. Of course, the 45 removal of the core is possible only in cases where the fiber coating the thread-like core would not itself be destroyed by the core removing agent. Likewise, if it is found desirable, the thread-like core may be rendered fire-proof, or it may be initially formed of fire-proof or water-proof mate-

rial, such as cellulose, artificial fiber or the like.

By the application of the novel insulating material hereinbefore disclosed, a conductor 55 of any shape or size may be covered in whole or in part with an efficient sheath of effective insulation, either fire-proof or waterproof in character and of any desired degree of thickness, and while the initial fiber coating applied to the foundation thread or filament is fluffy and apparently, but not actually, irregular in its disposition on the foundation thread, the ultimate insulating sheath is extremely compact and homogeneous and 60 uniform in disposition and insulating properties, so as to more nearly resemble a coating of plastic material rather than a fibrous sheath. An insulating sheath of this character is especially efficacious for conductors 65 to be wound in coil form on electrical apparatus in which it is desired to have the convolutions as close to each other as possible, consistent with the high degree of insulation 70 which the cellular character of the fibrous 75 material affords.

What I claim is:—

1. The combination of an electric conductor and an insulating sheath therefor, comprising a filamentary body having a complete superficial coating of fibers, said fiber coated filamentary body being wrapped about the conductor. 80

2. The combination of an electric conductor and an insulating sheath therefor, comprising successive convolutions of a filamentary body having a complete superficial coating of fibers, said fiber-coated body being applied to the surface of the conductor in a substantially uniform layer. 85 90

3. The combination of an electric conductor and an insulating sheath therefor, comprising a uniform layer of fiber-coated thread and a suitable binding material, the fibers constituting a complete superficial 95 coating for the thread.

In testimony whereof I affix my signature, in presence of two witnesses.

JOHN ALLEN HEANY.

Witnesses:

GEORGE H. DAVIS,  
VIOLA B. SMITH.